

June 30, 1942.

J. D. KENDALL ET AL

2,287,807

PHOTOGRAPHIC MATERIAL

Filed March 5, 1941



INVENTORS

John David Kendall  
Kenneth John Challis

BY *Lynn B. Morris*

ATTORNEY

## UNITED STATES PATENT OFFICE

2,287,807

## PHOTOGRAPHIC MATERIAL

John David Kendall and Kenneth John Challis,  
Ilford, England, assignors to Ilford Limited,  
Ilford, England, a British company

Application March 5, 1941, Serial No. 381,924  
In Great Britain April 12, 1940

5 Claims.

(CL. 95—8)

This invention relates to anti-halation layers for light-sensitive photographic elements and has particular reference to light-sensitive photographic materials which consist of a support, a light-sensitive layer on one side of the support and an anti-halation layer on the other side of the support.

The production of a satisfactory anti-halation layer on light-sensitive photographic material is a problem of some difficulty. A satisfactory anti-halation layer should adhere well to the support and should have no deleterious effect on the light sensitive layer, for example, when in contact therewith as in the case of the adjacent coils of film in a spool of film. Moreover, it is very important that the layer should be readily removed or decolourised during the processing of the light sensitive material; nevertheless it should preferably not be water soluble or it may mark or become tacky on touching with moist fingers, or dye present in the layer may stain the fingers when the photographic element is handled.

It has now been found that the mixed resin acids derived from tall oil form a combination which is of particular value as the carrier for an anti-halation dye or pigment. According to the present invention, therefore, there are provided photographic elements comprising a transparent support, a coating of light sensitive material on one face of the support, and an anti-halation layer on the other face of the support which comprises a continuous film formed from the mixed resin acids of tall oil and an anti-halation dye or pigment dispersed throughout said film.

The mixed resin acids obtained from tall oil readily form a continuous film when dissolved in a suitable solvent; cast as a layer and dried, and such layers do not deleteriously affect silver halide emulsion layers when brought into surface contact with them. Moreover, such layers adhere well to cellulose acetate and cellulose nitrate films and to glass and are readily dissolved or dispersed in the normal alkaline photographic developing solutions. It is a further advantage of such layers that they do not readily become tacky or mark when touched by moist hands and do not stain the hands when the photographic element is handled.

The mixed resin acids from tall oil may be obtained commercially as "Silvestic acid" but the commercial material is preferably purified before use, e. g. by dissolving the material in a 10% solution of sodium carbonate, filtering and reprecipitating the resin acids by the addition of an

acid (for example, hydrochloric acid) to the filtrate.

The anti-halation dye or pigment selected for any particular case must be one which is absorptive of light of wavelengths to which the photographic emulsion is sensitive. The invention may be applied for example to light sensitive film elements coated with panchromatic emulsions in which case a green or black dye is suitable, and to orthochromatic and non-colour-sensitised emulsions in which cases red and yellow dyes are respectively suitable.

Naturally occurring pigments may be employed in accordance with this invention since the whole anti-halation layer is removed during processing. However, it is preferable to employ organic dye-stuffs and particularly dyes which bleach out in the usual alkaline photographic developing solutions, e. g. dye of the triphenyl methane class such as Benzaurin (Schultz, Farbstoff-Tabellen No. 837), Acid Green G (Colour Index No. 666) Acid Magenta (Colour Index No. 692) and Lissamine Green S. F. (Colour Index No. 670 of Supplement). Mixtures of dyes or of pigments may be employed if desired.

In the production of the anti-halation layer of this invention a convenient method is to form a solution of the mixed resin acids in a suitable solvent, e. g. acetone or ethyl alcohol, and add to this sufficient of the anti-halation dye or pigment to give the desired tintorial strength, then to coat the resulting solution as a layer on the support layer of the photographic element, and then to dry the layer by evaporation of the solvent.

In the accompanying drawing a transparent support 1 has imposed thereon a light sensitive layer 2. On the reverse side of the support is imposed an antihalation layer 3 consisting of the resin acids of tall oil having dispersed there-through an antihalation material e. g. an anti-halation dye or pigment.

The following specific examples illustrate the invention:

## EXAMPLE 1

## Anti-halation layer for a photographic element carrying an orthochromatic emulsion

200 grams of the mixed resin acids from tall oil and 100 grams of Benzaurin are dissolved in a litre of acetone. Solution takes place in the cold. The solution is filtered and then coated and dried as a layer on one face of a glass plate which carries on the opposite face an orthochromatic silver halide emulsion. The anti-halation layer thus formed is firmly adherent to the glass

and is readily dissolved away in alkaline developer solutions.

EXAMPLE 2

*Anti-halation layer for a photographic element carrying a panchromatic silver halide emulsion*

200 grams of the mixed resin acids from tall oil and 50 grams of Acid Green G are dissolved in one litre of methylated spirit (74 O. P.). Solution takes place in the cold. After filtering the solution is coated and dried as an antihalation layer on one face of a glass plate which carries a panchromatic emulsion on the opposite face.

Instead of Acid Green G the same weight of Lissamine Green S. F. may be employed.

EXAMPLE 3

*Anti-halation layer for a photographic element carrying a panchromatic silver halide emulsion*

In this example an antihalation layer of somewhat deeper colour (i. e. of increased saturation) is produced, the solvent mixture being modified to take up the larger quantity of dyestuff.

200 grams of the mixed resin acids from tall oil is dissolved in a mixture of 800 ccs. of methylated spirit (74 O. P.) and 200 ccs. of ethylene glycol monomethyl ether. To the resulting solution is added 100 gms. of Acid Green G and the solution is shaken to facilitate solution. After filtering, the solution is coated and dried to form an antihalation layer as in Example 2.

EXAMPLE 4

*Anti-halation layer for a photographic element carrying an orthochromatic silver halide emulsion*

400 grams of the mixed resin acids from tall oil are dissolved in a mixture of 500 ccs. of methylated spirit (74 O. P.) and 500 ccs. of ethylene glycol monomethyl ether. To the resulting solution is added 100 grams of Acid Magenta and the solution shaken to facilitate solution. After filtering, the solution is coated and dried to form an anti-halation layer as in Example 2.

What we claim is:

1. A photographic element comprising a transparent support, a coating of light-sensitive material on one face of the support and an anti-halation layer on the other face of the support, 50

said antihalation layer comprising a continuous film of the mixed resin acids of tall oil and, dispersed throughout said film, a colouring matter which is absorptive of light of wavelengths to which the light-sensitive coating is sensitive.

2. A photographic element comprising a transparent support, a coating of light-sensitive material on one face of the support and an antihalation layer on the other face of the support, said 10 antihalation layer comprising a continuous film of the mixed resin acids of tall oil and, dispersed throughout said film, a dye which is absorptive of light wavelengths to which the light-sensitive coating is sensitive, and which is destroyed by 15 alkaline photographic developer solutions.

3. A photographic element comprising a transparent support, a coating of light-sensitive material on one face of the support and an anti-halation layer on the other face of the support, 20 said antihalation layer comprising a continuous film of the mixed resin acids of tall oil and, dispersed throughout said film, a dyestuff of the triphenyl methane class which is absorptive of light of wavelengths to which the light sensitive coating is sensitive, and which is destroyed by alkaline photographic developer solutions.

4. A photographic element, comprising a glass support, a coating of light-sensitive material on one face of the support and an antihalation layer 25 on the other face of the support, said antihalation layer comprising a continuous film of the mixed resin acids of tall oil and, dispersed throughout said film, a dyestuff of the triphenyl methane class which is absorptive of light of wavelengths to which the light sensitive coating is sensitive and which is destroyed by alkaline photographic developer solutions.

5. A photographic element comprising a transparent support, a light sensitive silver-halide emulsion layer on one face of the support and an antihalation layer on the other face of the support, said antihalation layer being composed of the mixed resin acids of tall oil having dispersed therethrough a dye which is absorptive of wavelengths to which the light sensitive layer is sensitive and which is destroyed by alkaline photographic developer solutions.

JOHN DAVID KENDALL.  
KENNETH JOHN CHALLIS.